

# United States Patent Office

3,019,145

Patented Jan. 30, 1962

1

3,019,145

## HIGH ENERGY HYDROCARBON FUEL CONTAINING MAGNESIUM ALLOYS

Lawrence Whitby, Midland, Mich., assignor to The Dow Chemical Company, Midland, Mich., a corporation of Delaware

No Drawing. Filed May 5, 1958, Ser. No. 732,790  
14 Claims. (Cl. 149—87)

This invention relates to high energy fuels, and more particularly to a high energy fuel comprising a hydrocarbon liquid and a magnesium product dispersed in said hydrocarbon and method for its preparation.

The importance of high energy fuel has increased considerably with the development of jet and rocket engines. To develop high speeds and high thrusts with rocket or jet engines high energy fuel is essential. In addition to the high energy content, the fuel must be chemically and physically stable. Also, it must be such that it can be easily stored and handled. Further the fuel must be readily ignitable and must be capable of being metered as a fluid into the combustion chamber of the engine without the need of complicated mechanical devices.

The heats of oxidation of certain light metals and metalloids, such as magnesium, aluminum, calcium, silicon, and boron, are so high either in terms of heat content per unit weight of fuel or per unit weight of oxygen, or both that they possess a great potential value in providing increased range and thrust when used as fuels in propulsion units such as jet, ram-jets, or after burners. In order to obtain complete and rapid combustion of the metals or metalloids, they must not only be introduced into the combustion zone in extremely fine state of subdivision, but means must be found for their production and handling in such finely divided state without hazard, since in the dry state they are pyrophoric.

It is, therefore, an object of this invention to provide a high energy fuel which will meet the requirements set forth above containing a magnesium alloy or a magnesium compound or mixtures thereof and a method for its preparation.

The high energy fuel of the invention comprises a hydrocarbon liquid, a dispersant dissolved in said liquid, and a friable low ductility magnesium containing alloy or compound, such as the brittle magnesium alloys of calcium, aluminum, or silicon, intermetallic compounds of magnesium with aluminum or calcium, and magnesium-boron compounds, dispersed therein as relatively equiaxed particles of less than 1.0 micron in size.

It has been discovered that within certain limits, as defined below, magnesium may be alloyed or combined with calcium, aluminum, silicon, or boron to form highly friable products that may be dispersed in hydrocarbon liquid by grinding, as by ball-milling. The solid metal is readily reduced by the grinding operation in the hydrocarbon liquid to particles of sub-micron dimensions. The resulting dispersions at concentrations of the dispersed phase of from 20 up to about 60% by weight form high energy fuels which are mobile, pumpable liquid mixtures, and readily ignitable.

The term "magnesium alloy" as used herein, means alloys containing magnesium in either major or minor proportions or in equal proportions with the other combustible constituents in the alloy.

Friable, low ductility magnesium products which have the desired friability to form relatively equiaxed particles upon grinding according to the invention are magnesium-aluminum alloys having an aluminum content from 14 to 85 weight percent, with the intermetallic compound  $Mg_{17}Al_{12}$  being particularly suitable; magnesium-calcium

2

alloys having a calcium content of from 15 to 80 weight percent with the range of calcium from the eutectic at 16.3 weight percent of calcium to about 45 weight percent, the intermetallic compound  $Mg_2Ca$ , being particularly suitable; magnesium-silicon alloys having a silicon content of from 3 to 60 weight percent; and magnesium-boron compounds corresponding to  $MgB_2$ ,  $MgB_4$ , and  $MgB_6$ . Of the friable, low ductility magnesium alloys or compounds, the magnesium-calcium alloys and the magnesium-aluminum alloys are preferred. These metals have a low density and burn with a high heat output.

A hydrocarbon liquid, such as benzene, toluene, and light petroleum fractions, such as gasoline, kerosene, diesel fuel, and fuel oils used at present as jet engine fuels, may be used as the hydrocarbon liquid in the high energy fuel. The term "light petroleum fraction" as used herein means the known petroleum fractions having an API gravity of 30 degrees or higher.

A dispersant chemically inert with respect to the magnesium alloy or compounds and soluble in the hydrocarbon liquid is incorporated into the dispersion. The dispersant adsorbs with preferred orientation upon the surface of the particles preventing agglomeration of the particles and thus considerably decreases the viscosity and improves the pumpability of the dispersion. Illustrative examples of suitable dispersants are lecithin; certain sorbitan esters, such as sorbitan trioleate; hydrocarbon liquid soluble substituted oxazolines, such as 2-heptadecenyl-4-methyl-4-methanol-2-oxazoline; dioctyl ester of sodium sulfosuccinate; polyoxyethylene lauryl ether; and propylene oxide stearyl ether. Other dispersing agents which are capable of assisting in dispersing of the magnesium product while being ground may be used provided they are substantially inert and unaffected by the magnesium alloy or compound used in the dispersion. With these dispersants, the dispersions have relatively low viscosities which remain remarkably constant over prolonged storage periods. Only a small amount of the dispersant need be used. However, the amount of the dispersant used is generally from 1 to 10 weight percent, based upon the weight of the hydrocarbon liquid. A preferred amount is from 4 to 6 weight percent. The dispersant is preferably added to the hydrocarbon liquid prior to comminuting the alloy. The high energy fuel is made most often by intermixing relatively large particles of the alloy with the hydrocarbon liquid and then comminuting the alloy in the mixture to the required particle size in admixture with the hydrocarbon liquid. The employment of a dispersant during the comminution results in a dispersion having smaller sized particles and considerably lower viscosity for a given concentration of the dispersed phase than that of a dispersion obtained without using a dispersant in the grinding operation. The dispersant, by being adsorbed upon the surface of the particles, prevents both pressure welding of the particles under the impact of grinding and also agglomeration of the particles.

Upon comminution of the friable low ductility magnesium alloys or compounds relatively equiaxed particles are obtained. These particles are readily combustible and when dispersed in the combustible hydrocarbon liquid in presence of a suitable dispersing agent do not greatly increase the viscosity of the liquid. When non-friable alloys or metals, for example magnesium or aluminum, are comminuted, relatively large plate-type particles are obtained which greatly increase the viscosity of the dispersion, compared to that of a dispersion having the same metal concentration but with metal particles in equiaxed form. Thus by using a friable alloy, yielding equiaxed particles on grinding, the concentration of the ground particles in the hydrocarbon liquid may be increased

up to about 60 weight percent without increasing the viscosity of the mixture to the extent that it cannot be easily pumped or handled.

In addition to obtaining a particular type of particle for controlling the viscosity of the dispersion, the particle size of the dispersed alloy must be less than 1 micron. The preferred particle size is in the range of 0.1 to 0.5 micron. It is clear that rapid and complete combustion is facilitated by extremely small particles and, moreover, smaller particles will settle less rapidly than larger particles. However, it is well-known that dispersions of solid particles in a continuous liquid phase will settle when the particles have a higher density than the liquid. This tendency may be offset by incorporating in the fuel a gelling agent which increases the thixotropy or pseudo-plasticity of the dispersions. Dispersions with thixotropic or pseudo-plastic rheological characteristics show a relatively high apparent viscosity at low shear rate, but the apparent viscosity is greatly reduced when the rate of shear is increased. Thus, such dispersions are highly viscous at rest, a condition which suppresses settling, but on shaking or stirring they become fluid. Small quantities of certain metal soaps, for example aluminum stearate and aluminum octoate, are suitable gelling agents for the above purpose. These may be incorporated into the dispersions by adding them as powders into the mixture prior to comminution or they may be mixed into the hydrocarbon liquid containing the dispersant using gentle heat to effect complete solution or dispersion rapidly. A suitable concentration of gelling agent has been found to be from 0.25% to 1% based on the weight of the hydrocarbon liquid.

To obtain magnesium alloy or compound particles of the required size, ball-milling may be used. Generally a ground or atomized powder or milling chips, such as very fine lathe turnings of the alloy, are mixed with an inert liquid containing a dispersant, such as previously described, and charged to a ball mill where the required size reduction is obtained. Any liquid inert to the magnesium alloy or compound may be used as the grinding fluid provided the dispersant is soluble therein. However, the hydrocarbon liquid which will be employed in the high energy fuel is most often used. Thus, the grinding and mixing operations are combined and the high energy fuel obtained after the comminution. Generally approximately equal weights of the magnesium product and hydrocarbon liquid are used. A fuel containing a smaller amount of the alloy may be simply obtained by diluting the concentrated comminuted product with more hydrocarbon liquid. If the grinding liquid used is not the hydrocarbon liquid which is to be a part of the fuel, the comminuted alloy is separated from the grinding fluid after the grinding, by various means apparent to those skilled in the art such as filtration, and intermixed with the hydrocarbon liquid which is desired to be a part of the fuel. Also, in order to obtain a dispersion in a liquid too viscous for effective ball-milling, without heating the ball mill, a dispersion in a low-boiling vehicle, such as benzene, may be prepared. This dispersion may be then mixed with the appropriate amount of the relatively vis-

cous liquid finally desired and the benzene distilled off from the mixture.

The time required to reduce the particle size of the alloy to the desired size may vary from a few hours to about 96 hours depending upon the particle size of the alloy charged to the mill and particular mill employed. For example, particles of the magnesium-aluminum compound  $Mg_{17}Al_{12}$  averaging 150 microns in size are reduced to a size in the range of 0.1 micron by grinding with kerosene for 96 hours in a ceramic mill with sintered alumina ( $Al_2O_3$ ) balls, and to about the same particle size in 48 hours by grinding in a steel mill with hardened steel balls.

The following examples further illustrate the invention but are not to be construed as limiting it thereto.

#### Example I

A high energy fuel according to the invention was prepared and the viscosity of this fuel compared to the viscosity of a dispersion made of pure magnesium.

In making this comparison, pellets of a magnesium alloy containing 17 percent calcium, the balance being magnesium, having a particle diameter in the range of 150 microns were intermixed with approximately an equal weight of kerosene which contained about 6 weight percent of sorbitan tri-oleate. This mixture was charged to a steel ball mill and ground therein for 48 hours when the particles of the alloy were reduced to a size in the range of 0.1 micron. The viscosity of the slurry so obtained was determined by a Brookfield torque-tube viscometer to be 1090 centipoises at 25° C. at 12 r.p.m. This fuel slurry was readily sprayed and ignitable and burned with intense heat.

For comparison, in place of the friable magnesium-calcium alloy, pellets of relatively pure magnesium also having a particle size of approximately 150 microns were used. The mixture of the magnesium and kerosene containing the sorbitan tri-oleate was ball-milled as above. After 48 hours of milling the particle size was found to be about 1.3 microns and the mixture was paste-like, its viscosity being too high to be measured by the method described above.

#### Example II

In a manner similar to that described in Example I, high energy fuels were prepared from two magnesium-calcium alloys one, A, containing 15 weight percent and the other, B, containing 45 weight percent of calcium respectively, the balance being magnesium. These fuels were compared to two similar dispersions obtained using magnesium-calcium alloys containing less than 15 weight percent of calcium. In the preparation of each of the fuels, the magnesium-calcium alloy as pellets having a particle size in the range of 150 microns was placed in the ball mill with kerosene and ball-milled for 48 hours. Other pertinent details of Example II are shown in the table below. It will be noted that with the magnesium-calcium alloys containing 8.4 and 3.6 weight percent calcium, respectively, and the balance magnesium, the dispersions obtained were paste-like.

| Magnesium Product Dispersed |                         | Amount of Solids in Fuel, Wt. Percent | Particle Size of Solids, Micron | Dispersant                                      | Amount of Dispersant, Wt. Percent, Based on Hydrocarbon Liquid | Brookfield Apparent Viscosity at 12 r.p.m., Centipoises |
|-----------------------------|-------------------------|---------------------------------------|---------------------------------|-------------------------------------------------|----------------------------------------------------------------|---------------------------------------------------------|
| Alloy                       | Composition             |                                       |                                 |                                                 |                                                                |                                                         |
| A.....                      | 15 Ca, Balance Mg.....  | 45                                    | 0.5                             | 2-heptadecinyl-4-methyl-4-methanol-2-oxazoline. | 6                                                              | 1,340.                                                  |
| B.....                      | 45 Ca, Balance Mg.....  | 80                                    | 0.2                             | do.....                                         | 6                                                              | 1,525.                                                  |
| Blank.....                  | 8.4 Ca, Balance Mg..... | 50                                    | 0.8                             | do.....                                         | 6                                                              | Paste-like.                                             |
| Blank.....                  | 3.6 Ca, Balance Mg..... | 50                                    | 1.0                             | do.....                                         | 6                                                              | Do.                                                     |

## Example III

In a manner similar to that described in Example I, high energy fuels of magnesium-silicon alloys one, C, and the other, D, containing 37 and 10 weight percent silicon respectively and the balance magnesium were prepared. These fuels were compared to a dispersion containing 2 weight percent silicon which gave a paste. Kerosene was used as the hydrocarbon liquid and the alloy particles having an initial particle size in the range of 150 microns were ball-milled for 48 hours. Other pertinent data of Example III are shown in table below:

| Magnesium Product Dispersed |                        | Amount of Solids in Fuel, Wt. Percent | Particle Size of Solids, Micron | Dispersant                               | Amount of Dispersant, Wt. Percent, Based on Hydrocarbon Liquid | Brookfield Apparent Viscosity at 12 r.p.m., Centipoises |
|-----------------------------|------------------------|---------------------------------------|---------------------------------|------------------------------------------|----------------------------------------------------------------|---------------------------------------------------------|
| Alloy                       | Composition            |                                       |                                 |                                          |                                                                |                                                         |
| C.....                      | 37 Si, Balance Mg..... | 50                                    | 0.5                             | Diocetyl ester of sodium sulfosuccinate. | 5                                                              | 650.                                                    |
| D.....                      | 10 Si, Balance Mg..... | 50                                    | 0.8                             | Sorbiton Trioleate.....                  | 4                                                              | 820.                                                    |
| Blank....                   | 2 Si, Balance Mg.....  | 50                                    | 1.0                             | Diocetyl ester of sodium sulfosuccinate. | 6                                                              | Paste-like.                                             |

## Example IV

In a manner similar to that described in Example I, four high energy fuels containing a magnesium-aluminum alloy were prepared. The magnesium-aluminum alloys used contained 15, 32, 45, and 67 weight percent aluminum respectively and the remainder magnesium. Pertinent details and data are shown in the table below:

| Magnesium Product Dispersed | Amount of Solids in Fuel, Wt. Percent | Particle Size of Solids, Micron | Dispersant                                      | Amount of Dispersant, Wt. Percent, Based on Hydrocarbon Liquid | Brookfield Apparent Viscosity at 12 r.p.m. |
|-----------------------------|---------------------------------------|---------------------------------|-------------------------------------------------|----------------------------------------------------------------|--------------------------------------------|
| 15 Al, Balance Mg.....      | 55                                    | 0.7                             | Sorbiton trioleate.....                         | 6                                                              | 950                                        |
| 32 Al, Balance Mg.....      | 50                                    | 0.2                             | 2-heptadicinyl-4-methyl-4-methanol-2-oxazoline. | 6                                                              | 1,530                                      |
| 45 Al, Balance Mg.....      | 60                                    | 0.1                             | do.....                                         | 5.4                                                            | 2,210                                      |
| 67 Al, Balance Mg.....      | 50                                    | 0.2                             | Lecithin.....                                   | 6                                                              | 1,720                                      |

What is claimed is:

1. A fluid high energy fuel which consists essentially of a combustible hydrocarbon liquid containing a dispersant dissolved therein and a friable low ductility magnesium product selected from the group consisting of alloys and intermetallic compounds of magnesium with calcium, aluminum, silicon, and boron, in the form of relatively equiaxed particles less than 1.0 micron in size in an amount of from 20 up to 60 weight percent of the fuel, said dispersant being chemically inert with respect to the magnesium product and adsorbed upon surface of said equiaxed particles preventing agglomeration of said particles.

2. A fluid high energy fuel according to claim 1 where-in the hydrocarbon liquid is a light petroleum fraction containing from 1 to 10 weight percent of a dispersant dissolved therein.

3. A fluid high energy fuel, which consists essentially of a light petroleum fraction containing from 1 to 10 weight percent of a dispersant dissolved therein and a magnesium-calcium alloy containing from 85 to 20 weight percent magnesium and from 15 to 80 weight percent calcium in the form of relatively equiaxed particles of less than 1 micron in size in an amount of from 20 to 60 weight percent of the fuel, said dispersant being chemically inert with respect to the magnesium product and adsorbed upon surface of said equiaxed particles preventing agglomeration of said particles.

4. A fluid high energy fuel, which consists essentially of kerosene containing from 4 to 6 weight percent of a

dispersant dissolved therein and a magnesium-calcium alloy containing from 85 to 55 weight percent of magnesium and from 15 to 45 weight percent calcium in the form of relatively equiaxed particles of from 0.1 to 0.5 micron in size in an amount of from 20 to 60 weight percent of the fuel, said dispersant being chemically inert with respect to the magnesium product and adsorbed upon surface of said equiaxed particles preventing agglomeration of said particles.

10 5. A fluid high energy fuel, which consists essentially of a light petroleum fraction containing from 1 to 10

weight percent of a dispersant dissolved therein and a magnesium-aluminum alloy containing from 15 to 86 weight percent magnesium and 85 to 14 weight percent aluminum dispersed in said light petroleum fraction as relatively equiaxed particles of less than 1 micron in size in an amount of from 20 to 60 weight percent of the fuel, said dispersant being chemically inert with re-

spect to the magnesium product and adsorbed upon surface of said equiaxed particles preventing agglomeration of said particles.

50 6. A fluid high energy fuel according to claim 5 where-in the light petroleum fraction is kerosene containing from 4 to 6 weight percent of sorbitan trioleate dissolved therein, as a dispersant, the magnesium-aluminum alloy is the intermetallic compound  $Mg_{17}Al_{12}$ , and the particle size is in the range of 0.1 to 0.5 micron.

60 7. A fluid high energy fuel, which consists essentially of a light petroleum fraction containing from 1 to 10 weight percent of a dispersant dissolved therein and a magnesium-silicon alloy containing from 40 to 97 weight percent magnesium and 3 to 60 weight percent silicon dispersed in said light petroleum fraction as relatively equiaxed particles of less than 1 micron in size in an amount of from 20 to 60 weight percent of the fuel, said dispersant being chemically inert with respect to the magnesium product and adsorbed upon surface of said equiaxed particles preventing agglomeration of said particles.

65 8. A process for the preparation of high energy fuel, which comprises comminuting a friable low ductility magnesium product selected from the group consisting of alloys and intermetallic compounds of magnesium with calcium, aluminum, silicon, and boron, in an organic liquid medium inert to the magnesium product and containing a dispersant dissolved therein until the particle size of the product is reduced to less than 1 micron separating the comminuted particles of the magnesium product from the organic liquid medium and intermixing the

particles of said magnesium product in a hydrocarbon liquid in proportions such that the resulting mixture contains from 20 to 60 weight percent of the magnesium product.

9. A process for the preparation of a high energy fuel, which comprises intermixing a hydrocarbon liquid containing a soluble dispersant with a friable low ductility magnesium product selected from the group consisting of alloys and intermetallic compounds of (1) magnesium-aluminum mixtures containing from 14 to 85 percent aluminum, (2) magnesium-calcium mixtures containing from 15 to 80 weight percent calcium, and (3) magnesium-silicon containing from 3 to 60 weight percent silicon and intermetallic compounds of magnesium-boron corresponding to the formula  $MgB_2$ ,  $MgB_4$  and  $MgB_6$ , in proportion such that the resulting mixture contains from 20 to 60 weight percent of said magnesium product and comminuting the magnesium product while in the liquid until the particle size of the magnesium product is reduced to from 0.1 to 0.5 micron, said dispersant being chemically inert with respect to the magnesium product and adsorbed upon surface of said equiaxed particles preventing agglomeration of said particles.

10. A process according to claim 9 wherein the hydrocarbon liquid is a light petroleum fraction containing from 1 to 10 weight percent of sorbitan trioleate dissolved therein, as a dispersant.

11. A process according to claim 10 wherein the friable low ductility magnesium product is a magnesium-

calcium alloy containing from 85 to 20 weight percent magnesium and from 15 to 80 weight percent calcium.

12. A process according to claim 10 wherein the friable low ductility magnesium product is a magnesium-aluminum alloy containing from 15 to 86 weight percent magnesium and from 14 to 85 weight percent aluminum.

13. A process according to claim 10 wherein the friable low ductility magnesium product is a magnesium boron compound.

14. A mobile, pumpable liquid high energy fuel according to claim 4 wherein the dispersant is 2-heptadecinyl-4-methyl-4-methanol-2-oxazoline.

#### References Cited in the file of this patent

#### UNITED STATES PATENTS

|           |               |               |
|-----------|---------------|---------------|
| 1,532,930 | O'Neill       | Apr. 7, 1925  |
| 2,477,549 | Van Loenen    | July 26, 1949 |
| 2,573,471 | Malina et al. | Oct. 30, 1951 |
| 2,579,257 | Hansley       | Dec. 18, 1951 |
| 2,890,108 | Toulmin       | June 9, 1959  |

#### OTHER REFERENCES

25 Anderton: Aviation Week, Nov. 12, 1956, pages 51, 53, 55, 43rd Report of National Advisory Committee for Aeronautics (1957), pages 2-4.

Frazier: Proceedings 14th Annual Meeting, Metal Powder Association, April 21-3, 1958, pages 65-70.